

G. F. Sack,  
Casting Letters and Ornaments.  
No 80,567. Patented Aug. 4, 1868.

Fig 1.



Fig 2.



Witnesses.

Chas Goldavery  
  
Joseph Goldavery  


Inventor.  
George F. Sack

# United States Patent Office.

GEORGE F. SACK, OF NEW YORK, N. Y.

*Letters Patent No. 80,567, dated August 4, 1868.*

## IMPROVEMENT IN MOULDS FOR CASTING LETTERS, &c.

The Schedule referred to in these Letters Patent and making part of the same.

Be it known that I, GEORGE F. SACK, of the city and county of New York, have invented a new and improved Mode of Producing Metal Letters and Ornaments; and I do hereby declare the following to be a full, clear, and exact description of my said invention, reference being had to the accompanying drawings.

I first make a pattern of the letter or ornament desired, and grinding a smooth surface upon the soft side of a piece of sepiæ, (cuttle-fish,) and I lay my pattern on a convenient spot of the smoothed surface, and press it thereon until the pattern is embedded in the sepiæ.

The mould produced thereby is an accurate impression of the pattern, showing the finest lineaments thereof. The pattern is then removed. The counterpart to the mould is made of another piece of sepiæ in the same manner. A little channel is cut out in the sepiæ for the infusion of the melted metal. The two parts of the mould are fitted together, and the melted metal is poured in the mould. When cooled, the sepiæ is removed, and the casting will be found to be a perfect reproduction of the pattern, requiring but little polishing to be rendered fit for application to its purpose.

By this means, letters or trinkets are produced; which, with other moulds, could be rendered so neat and ornamental only by being chased or engraved.

After the sepiæ is removed, the casting may be enamelled, burnished, gilded, &c.

In the accompanying drawing—

Figure 1 represents the mould, produced in the manner described, and

Figure 2 the letter E cast therein.

I claim as my invention, and desire to secure by Letters Patent of the United States—

A mould for casting letters and ornaments, which will retain an accurate impression of the most delicate lineaments of the pattern, made of a sepiæ or cuttle-fish bone, in the manner substantially as herein described, and for the purpose mentioned.

GEORGE F. SACK.

Witnesses:

CHAS. GOLDZIER,

JOSEPH GOLDSCHIEDER.